

July 26, 1960

G. H. JONKER ET AL

2,946,753

FERROMAGNETIC MATERIAL

Filed Aug. 9, 1956

5 Sheets-Sheet 1



FIG. 1

INVENTORS

GERARD HENRICH JONKER  
HENRICUS PETRUS JOHANNES WIJN  
POUL BERNARD BRAUN

BY

*Frederick Vogel*

AGENT

July 26, 1960

G. H. JONKER ET AL  
FERROMAGNETIC MATERIAL

2,946,753

Filed Aug. 9, 1956

5 Sheets-Sheet 2



FIG. 2

INVENTORS  
GERARD HEINRICH JONKER  
HENRICUS PETRUS JOHANNES WIJN  
POUL BERNARD BRAUN

BY

*Fred G. Vogel*

AGENT

July 26, 1960

G. H. JONKER ET AL  
FERROMAGNETIC MATERIAL

2,946,753

Filed Aug. 9, 1956

5 Sheets-Sheet 3



FIG.3

INVENTORS

GERARD HEINRICH JONKER  
HENRICUS PETRUS JOHANNES WIJN  
POUL BERNARD BRAUN

BY

*Fred M. Vogel*  
AGENT

July 26, 1960

G. H. JONKER ET AL  
FERROMAGNETIC MATERIAL

2,946,753

Filed Aug. 9, 1956

5 Sheets-Sheet 4



INVENTORS  
GERARD HEINRICH JONKER  
HENRICUS PETRUS JOHANNES WIJN  
POUL BERNARD BRAUN

BY

*Free L. Vogel*

AGENT

July 26, 1960

G. H. JONKER ET AL  
FERROMAGNETIC MATERIAL

2,946,753

Filed Aug. 9, 1956

5 Sheets-Sheet 5



INVENTORS  
GERARD HEINRICH JONKER  
HENRICUS PETRUS JOHANNES WIJN  
POUL BERNARD BRAUN  
BY *Frederick M. Vogel*  
AGENT

# United States Patent Office

2,946,753

Patented July 26, 1960

1

2,946,753

## FERROMAGNETIC MATERIAL

Gerard Heinrich Jonker, Henricus Petrus Johannes Wijn, and Poul Bernard Braun, all of Eindhoven, Netherlands, assignors, by mesne assignments, to North American Philips Company, Inc., New York, N.Y., a corporation of Delaware

Filed Aug. 9, 1956, Ser. No. 603,136

Claims priority, application Netherlands Aug. 10, 1955

8 Claims. (Cl. 252—62.5)

Our invention relates to oxidic ferromagnetic materials, to methods of preparing these materials and to bodies made from these materials.

Oxidic ferromagnetic materials which exhibit high values of initial permeability are known in the art. All these materials show a decrease of the initial permeability in a certain frequency range the position of which in the frequency scale is related to the low-frequency value of the initial permeability. The initial permeability decreases in a frequency range the position of which in the frequency scale is higher in proportion as the value of the initial permeability at low-frequency is lower. Thus the cores formed from these materials are not too satisfactory for use at high frequencies.

The principal object of our invention, therefore, is to provide a new and novel class of oxidic ferromagnetic materials the initial permeability of which decreases in a much higher positioned frequency range than in the known materials with an equal low frequency value of the initial permeability.

Another object of our invention is to provide oxidic ferromagnetic materials which have initial permeabilities of more and often materially more than 2 at frequencies of about 50 mc./s. and often considerably higher frequencies and which exhibit low losses.

Still another object of our invention is to provide oxidic ferromagnetic materials which may serve as materials for magnetic bodies e.g. cores at frequencies of about 50 mc./s and often considerably higher frequencies.

These and other objects of our invention will be apparent as the specification progresses.

According to our invention we have found new and novel materials having a composition  $BaM^{II}Fe_6^{III}O_{11}$  wherein  $M^{II}$  is at least one divalent metal selected from the group consisting of Mn, Fe, Co, Ni, Cu, Zn and Mg. In the aforesaid formula Ba may be replaced partly by similar ions, for example Sr, Ca and Pb, since the Ba may be replaced at a maximum for half by Sr or at a maximum for one quarter by Ca or Pb. Of course the Ba-ion, may, as an alternative, be replaced partly by a combination of similar ions. Moreover, the  $Fe^{III}$  ions may be replaced for at most one tenth by Cr and/or Al-ions. Thus, the formula for these materials may be restated as follows:



In the formula  $M^{II}$  represents one of the aforesaid divalent metals and the subscripts have the following value

- a less than 0.5
- b less than 0.25
- c less than 0.25
- (b+c) less than 0.25
- e less than 0.6
- f less than 0.6
- (e+f) less than 0.6

All these materials have initial permeabilities which do not decrease substantially up to very high frequencies.

2

They have initial permeabilities of more and often materially more than 2 at frequencies of about 50 mc./s. and often considerably higher frequencies. Since they are basically oxidic in nature they are characterized by high ohmic resistances so that eddy current losses are negligibly small. In addition to having greatly improved initial permeabilities at high frequencies, particularly above 50 mc./s., the materials of our invention exhibit relatively low residual loss factors ( $\tan \delta$ ) at frequencies above 50 mc./s.

The novel materials of our invention have a rhombohedral crystal structure of which the unit cell in the hexagonal crystal system has a coaxis of about 43.5 Å and an axis of about 5.9 Å.

While the entire class of our novel materials have improved magnetic properties, particularly in regard to their initial permeabilities, we have found that materials having a composition  $BaZn_xMg_yMe^{II}(1-x-y)Fe_6^{III}O_{11}$ , where in  $0 \leq x \leq 1$ ,  $0 \leq y \leq 1$  and  $0 < (x+y) \leq 1$  and wherein  $Me^{II}$  is at least one divalent metal selected from the group consisting of Mn, Fe, Co, Ni and Cu, in which formula the Ba may be replaced in the aforesaid manner, have even further improved initial permeabilities.

We prepare the novel materials of our invention by heating at a temperature of more than 1000° C. a finely divided mixture of metallic oxides in a ratio approximately corresponding to that of the metals in the materials of our invention. Alternatively instead of a metallic oxide we may use a material which forms an oxide when heated. As these oxide-forming materials we may use carbonates, oxalates and acetates of the metals. Moreover, instead of metallic oxides we may use one or more preformed reaction products of at least two of the metallic oxides.

Preferably we prepare the novel materials of our invention by heating at a temperature of between 1150° C. and 1300° C. a finely divided mixture of metallic oxides and/or oxide-forming materials and/or reaction products of metallic oxides, in a ratio approximately corresponding to that of the metals in the materials of our invention.

As a preformed reaction product of at least two of the metallic oxides we preferably use an iron-containing reaction product, which has been produced at low temperature, preferably below 1100° C., and which has a crystal structure corresponding with that of the mineral magnetoplumbite, for example  $Ba_xSr_{(1-x)}Fe_{12}O_{19}$ , where in  $0 \leq x \leq 1$ .

If necessary the mixture of oxides and/or equivalent materials may be presintered, usually at a relatively low temperature of about 900° C. to 1200° C., the presintered material being reground and resintered several more times if desired before being subjected to the higher temperatures of the process.

In order to facilitate the sintering operation of our process we may include various flux agents, for example silicates such as pentonite or fluorides such as calcium-fluoride in an amount of from 0.25% to 5% in the starting mixtures.

Bodies of desired shape may be formed by sintering the starting mixtures directly in the desired shape. Alternatively bodies of desired shape may be formed by regrinding the sintered material of our invention or the presintered material, molding the resultant powder into the desired shape and sintering the molded product if necessary. A binder such as water, a solution of nitrocellulose or a solution of carboxymethylcellulose may be added to the powdered mixtures before molding if necessary.

In a further embodiment of the invention the finely divided material of our invention is molded to form a

body of the desired shape by pressing the relative material together with a binding agent which is capable of being hardened (for example a polyester resin) or an ethoxylin resin followed by hardening the molded body.

Our invention will now be described in greater detail with reference to the following examples and drawing.

In the drawing, Figs. 1 to 5 are graphs showing the relationship between the values of the real portion of initial permeability,  $\mu'$ , and the values of the loss factor,  $\tan \delta$ , to frequency for various embodiments of our invention.

The relationship between the loss factor  $\tan \delta$  and the real portion of initial permeability,  $\mu'$ , will be apparent from the following explanation which forms no part of our invention and which is not to be used in any way to limit the scope of our invention:

The term  $\mu''$  as used herein may be explained as follows: A sinusoidally alternating magnetic field with small amplitude will produce a similarly varying inductance in a ferromagnetic body but due to ferromagnetic losses there will be a phase difference between the magnetic field and the inductance. Thus the permeability of the ferromagnetic body,  $\mu$ , may be represented by a complex magnitude  $\mu = \mu' - j\mu''$ . The real portion of permeability,  $\mu'$ , is in phase with the field applied while the other lags in phase by  $90^\circ$  with respect to the applied field. The loss factor "tan  $\delta$ " can then be defined as

$$\tan \delta = \frac{\mu''}{\mu'}$$

#### Example I

Mixtures having the following compositions were produced:

- (1) 98.7 gs. of BaCO<sub>3</sub>, 245.0 gs. of Fe<sub>2</sub>O<sub>3</sub>, and 46.3 gs. of MgCO<sub>3</sub>,
- (2) 98.7 gs. of BaCO<sub>3</sub>, 245.0 gs. of Fe<sub>2</sub>O<sub>3</sub>, and 64.9 gs. of CoCO<sub>3</sub>,
- (3) 98.7 gs. of BaCO<sub>3</sub>, 245.0 gs. of Fe<sub>2</sub>O<sub>3</sub>, and 63.7 gs. of NiCO<sub>3</sub>,
- (4) 98.7 gs. of BaCO<sub>3</sub>, 245.0 gs. of Fe<sub>2</sub>O<sub>3</sub>, and 40.8 gs. of ZnO.

Of the raw materials the BaCO<sub>3</sub> was substantially pure, the Fe<sub>2</sub>O<sub>3</sub> contained 68.4% by weight of iron, the MgCO<sub>3</sub> 26.2% by weight of magnesium, the CoCO<sub>3</sub> 45.3% by weight of cobalt, the NiCO<sub>3</sub> 46.1% by weight of nickel and the ZnO 78.4% by weight of zinc.

These mixtures were ground for 16 hours with ethyl alcohol in a chromium-plated iron ball mill. The dried powders were then presintered for two hours at 1050° in oxygen. The reaction products were ground for 16 hours. To these dried powders, a small amount of water was then added and rings having an outer diameter of about 35 mms., an inner diameter of about 25 mms. and a height of about 4 mms. were moulded at a pressure of 1000 kgs./cm.<sup>2</sup>. These rings were sintered for two hours in oxygen and then cooled to room temperature within about 4 hours. For the magnesium-, cobalt- and nickel-containing compounds the sintering temperature was 1260° C., and for the zinc-containing compound the sintering temperature was 1240° C. X-ray examination showed that in this manner comparatively pure compounds having desired structure were obtained. Also small quantities of compounds having a spinel crystal structure (probably MgFe<sub>2</sub>O<sub>4</sub>, CoFe<sub>2</sub>O<sub>4</sub>, NiFe<sub>2</sub>O<sub>4</sub>, ZnFe<sub>2</sub>O<sub>4</sub>) and also a small quantity of BaFe<sub>2</sub>O<sub>4</sub> were formed. The properties of this series of compounds are indicated in the table under Nos. 1 to 4.

#### Example II

A number of rings of the zinc-containing material, described in Example I, were sintered for only half an hour at 1200° C. in oxygen and then cooled to room temperature within about one hour. The properties of these rings are indicated in the table under No. 5.

#### Example III

A mixture of 26.0 gs. of BaCO<sub>3</sub>, 60.0 gs. of Fe<sub>2</sub>O<sub>3</sub> and 9.5 gs. of NiO was ground with ethyl alcohol in a porcelain ball mill. The dried mixture was presintered for 15 hours at 1100° C. in air. This reaction product was then ground again for half an hour. From this material rings were molded at a pressure of 1000 kgs./cm.<sup>2</sup> having an outer diameter of about 35 mms., an inner diameter of 25 mms. and a height of about 4 mms., after the addition of a small quantity of a solution of nitrocellulose as an organic binder. These rings were sintered in oxygen at a temperature of 1290° C. and then cooled to room temperature within about 5 hours. An X-ray examination proved that the material thus obtained consisted almost entirely of the desired compound BaNi<sup>II</sup>Fe<sub>6</sub><sup>III</sup>O<sub>11</sub>, whilst a small quantity of BaFe<sub>2</sub>O<sub>4</sub> was formed as a second phase. The properties of the rings are indicated in the table under No. 6.

#### Example IV

Mixtures having the following compositions were produced:

- (7) 98.7 gs. of BaCO<sub>3</sub>, 245.0 gs. of Fe<sub>2</sub>O<sub>3</sub>, 9.2 gs. of MgCO<sub>3</sub> and 32.6 gs. of ZnO,
- (8) 98.7 gs. of BaCO<sub>3</sub>, 245.0 gs. of Fe<sub>2</sub>O<sub>3</sub>, 13.0 gs. of CoCO<sub>3</sub> and 32.6 gs. of ZnO,
- (9) 98.7 gs. of BaCO<sub>3</sub>, 245.0 gs. of Fe<sub>2</sub>O<sub>3</sub>, 38.2 gs. of NiCO<sub>3</sub> and 16.3 gs. of ZnO.

These mixtures were pre-treated as described in Example I and rings were molded at a pressure of 1000 kgs./cm.<sup>2</sup> having an outer diameter of about 35 mms., an inner diameter of about 25 mms. and a height of about 4 mms. These rings were heated in oxygen for two hours at 1280° C. and then cooled slowly. An X-ray examination showed that the reaction products formed consisted almost entirely of the desired compounds



40 BaZN<sub>0.8</sub>Co<sub>0.2</sub>Fe<sub>6</sub>O<sub>11</sub>, BaZN<sub>0.6</sub>Ni<sub>0.4</sub>Fe<sub>6</sub>O<sub>11</sub>, respectively. Also small quantities of compounds having a spinel crystal structure (probably MgFe<sub>2</sub>O<sub>4</sub>, CoFe<sub>2</sub>O<sub>4</sub>, NiFe<sub>2</sub>O<sub>4</sub>, ZnFe<sub>2</sub>O<sub>4</sub>) were formed. The properties of these compounds are indicated in the table under Nos. 7, 8 and 9.

#### Example V

A mixture of barium carbonate, strontium carbonate, zinc oxide and ferric oxide in a ratio in accordance with the formula Ba<sub>0.5</sub>Sr<sub>0.5</sub>ZnFe<sub>6</sub>O<sub>11</sub> was ground with ethyl alcohol in a porcelain ball mill. The dried mixture was presintered for 15 hours at 1100° C. in air. This reaction product was then ground again for half an hour. After the addition of a small quantity of a solution of carboxymethylcellulose as an organic binder, rings were molded from this material at a pressure of 1000 kgs./cm.<sup>2</sup>, the rings having an outer diameter of about 35 mms., an inner diameter of about 25 mms. and a height of about 4 mms. These rings were sintered in oxygen at a temperature of 1230° C. and then cooled to room temperature within about 4 hours. By X-ray examination it was found that in this manner a comparatively pure compound of the desired structure was obtained. The properties of the rings are indicated in the table under No. 10.

#### Example VI

In the manner described in Example V, starting from a mixture of barium carbonate, calcium carbonate, zinc oxide and ferric oxide in a ratio in accordance with the formula Ba<sub>0.75</sub>Ca<sub>0.25</sub>ZnFe<sub>6</sub>O<sub>11</sub>, a material was produced which consisted almost entirely of the desired compound, as was proved by X-ray examination, whilst a small quantity of crystals with spinel crystal structure (probably ZnFe<sub>2</sub>O<sub>4</sub>) was obtained as a second phase. The properties of this compound are indicated in the table under No. 11.

## Example VII

In the manner described in Example V, however, with the difference that heating was performed at 1200° C. instead of 1230° C., starting from a mixture of barium carbonate, lead carbonate, zinc oxide and ferric oxide in a ratio in accordance with the formula



a material was produced, which consisted, as was proved by X-ray examination, almost entirely of the desired compound, whilst a small quantity of crystals with spinel crystal structure (probably  $\text{ZnFe}_2\text{O}_4$ ) was obtained as a second phase. The properties of this compound are indicated in the table under No. 12.

## Example VIII

From  $\text{BaCO}_3$  and  $\text{Fe}_2\text{O}_3$  in the molecular ratio of 1:5.6 by heating the mixture for 15 hours at 900° C. a material was produced which consisted primarily of the compound  $\text{BaFe}_{12}\text{O}_{19}$ . 33 gs. of this material was mixed with 5.2 gs. of  $\text{BaCO}_3$ , 2.26 gs. of  $\text{ZnO}$  and 21.9 gs. of  $\text{CoCO}_3$ , which corresponds to the desired compound



The mixture was ground for one hour with ethyl alcohol in a porcelain ball mill and after drying it was presintered for two hours at 1100° C. in oxygen. After regrinding, the product was shaped in the form of rings at a pressure of 1000 kgs./cm.<sup>2</sup>, which were fired at 1240° C. in oxygen. By X-ray examination it was found that indeed the desired compound was obtained. The properties of the rings are indicated in the table under No. 13.

## Example IX

The compounds  $\text{BaFe}_{12}\text{O}_{19}$ ,  $\text{BaFe}_2\text{O}_4$  and  $\text{ZnFe}_2\text{O}_4$  were

35 ized.

| No. | Main Constituent                                             | $d$ ,<br>g./cm. <sup>3</sup> | $\rho$ ,<br>Ω cm. | $\mu'$ ,<br>Low<br>frequency | $\mu'$ ,<br>50<br>Mc./s. | $\mu'$ ,<br>500<br>Mc./s. | Figure |
|-----|--------------------------------------------------------------|------------------------------|-------------------|------------------------------|--------------------------|---------------------------|--------|
| 1   | $\text{BaMgFe}_8\text{O}_{11}$                               | 3.3                          | $10^7$            | 11                           | 10                       | 10                        | 1      |
| 2   | $\text{BaCoFe}_8\text{O}_{11}$                               | 5.0                          | $10^4$            | 4                            | 4                        | 3.5                       | 2      |
| 3   | $\text{BaNiFe}_8\text{O}_{11}$                               | 4.0                          | $10^3$            | 5                            | 5                        | 5                         | —      |
| 4   | $\text{BaZnFe}_8\text{O}_{11}$                               | 4.6                          | $10^4$            | 32                           | 21                       | 12                        | 3      |
| 5   | $\text{BaZnFe}_8\text{O}_{11}$                               | 3.4                          | $10^3$            | 12                           | 8.2                      | 6                         | 4      |
| 6   | $\text{BaZnFe}_8\text{O}_{11}$                               | 4.2                          | $10^4$            | 6                            | 5                        | 4                         | —      |
| 7   | $\text{BaZn}_{0.8}\text{Mg}_{0.2}\text{Fe}_8\text{O}_{11}$   | 4.7                          | $10^3$            | 25                           | 19                       | 11                        | —      |
| 8   | $\text{BaZn}_{0.8}\text{Co}_{0.2}\text{Fe}_8\text{O}_{11}$   | 4.8                          | $10^2$            | 15                           | 13                       | 10                        | —      |
| 9   | $\text{BaZn}_{0.8}\text{Ni}_{0.2}\text{Fe}_8\text{O}_{11}$   | 4.6                          | $10^3$            | 20                           | 19                       | 12                        | —      |
| 10  | $\text{Ba}_{0.8}\text{Sr}_{0.2}\text{ZnFe}_8\text{O}_{11}$   |                              |                   | 15.4                         | 14.7                     | 5.3                       | —      |
| 11  | $\text{Ba}_{0.75}\text{Ca}_{0.25}\text{ZnFe}_8\text{O}_{11}$ |                              |                   | 12.3                         | 9.2                      | 5.7                       | —      |
| 12  | $\text{Ba}_{0.75}\text{Pb}_{0.25}\text{ZnFe}_8\text{O}_{11}$ |                              |                   | 32.6                         | 25.1                     | 10.1                      | —      |
| 13  | $\text{BaCo}_{0.8}\text{Zn}_{0.5}\text{Fe}_8\text{O}_{11}$   |                              |                   | 7.9                          | 7.2                      | 7.0                       | —      |
| 14  | $\text{BaZnFe}_8\text{O}_{11}$                               |                              |                   | 14.2                         | 9.3                      | 7.2                       | —      |
| 15  | $\text{BaZn}_{0.8}\text{Al}_{0.2}\text{Fe}_8\text{O}_{11}$   |                              |                   | 13.8                         | 12.1                     | —                         | —      |
| 16  | $\text{BaZn}_{0.8}\text{Cr}_{0.2}\text{Fe}_8\text{O}_{11}$   |                              |                   | 5.4                          | 4.2                      | —                         | —      |

previously produced by presintering mixtures of correctly chosen proportions of  $\text{BaCO}_3$  and  $\text{Fe}_2\text{O}_3$ ,  $\text{BaCO}_3$  and  $\text{Fe}_2\text{O}_3$  and  $\text{ZnO}$  and  $\text{Fe}_2\text{O}_3$  at 1150° C. in air. Then a mixture of 15.72 gs. of  $\text{BaFe}_{12}\text{O}_{19}$ , 20.88 gs. of  $\text{BaFe}_2\text{O}_4$  and 16.06 gs. of  $\text{ZnFe}_2\text{O}_4$ , which corresponds to the desired compound  $\text{BaZnFe}_8\text{O}_{11}$ , was ground for 4 hours with ethyl alcohol in a vibration mill, after which rings were molded from this product at a pressure of 1000 kgs./cm.<sup>2</sup>; these rings were fired for one hour at 1180° C. in oxygen. X-ray examination proved that in this manner a fairly pure compound with the desired structure was obtained. The properties of the rings are indicated in the table under No. 14.

## Example X

From  $\text{BaCO}_3$  and  $\text{Fe}_2\text{O}_3$  in the molecular ratio of 1:5.6 by heating the mixture for 15 hours at 900° C., a material was produced which consisted primarily of the compound  $\text{BaFe}_{12}\text{O}_{19}$ . 32.4 gs. of this material was mixed with 6.05 gs. of  $\text{BaCO}_3$ , 4.9 gs. of  $\text{ZnO}$  and 1.54 gs. of  $\text{Al}_2\text{O}_3$ , which corresponds to the desired compound



32.4 gs. of the material was mixed with 6.05 gs. of  $\text{BaCO}_3$ , 4.9 gs. of  $\text{ZnO}$  and 2.33 gs. of  $\text{Cr}_2\text{O}_3$ , which corresponds to the desired compound  $\text{BaZnFe}_{5.5}\text{Cr}_{0.5}\text{O}_{11}$  (16). The mixtures were ground for one hour with ethyl alcohol in a porcelain ball mill and after drying they were presintered for two hours at 1000° C. in oxygen. After regrinding, the reaction products were molded to form rings at a pressure of 1000 kgs./cm.<sup>2</sup>, which were fired at 1250° C. in oxygen. X-ray examination proved that, indeed, the desired compounds were formed. The properties of the rings are indicated in the table under Nos. 15 and 16.

Many other similar compounds may be produced in an analogous manner.

15 In the following table, in column 2, under the heading of "Main Constituent," chemical formulae are indicated, which were derived from the compositions of the starting mixtures and from the X-ray examinations. All measuring results were obtained by carrying out measurements on rings in a demagnetized state at room temperature by the method described by C. M. van der Burgt, M. Gevers and H. P. J. Wijn in "Philips Technical Review," 14, 245 (1952-1953).

The graphs of Figs. 1 to 5 show the relationship between the real portion of the initial permeability,  $\mu'$ , and  $\tan \delta$  to frequency for the products designated in the table under Nos. 1, 2, 4, 5 and 6 respectively. In these graphs the values of  $\mu'$  and  $\tan \delta$  are plotted along the ordinates and the values of the frequencies are plotted along the abscissa. In addition the graph of Fig. 4, which pertains to product No. 5, shows by means of broken lines the properties of the product after it has been magnetized in a strong magnetic field which was subsequently neutralized.

25 30 35

While we have described our invention in connection with specific embodiments and applications, other modifications thereof will be readily apparent to those skilled in this art without departing from the spirit and scope of the invention as defined in the appended claims.

What we claim is:

1. A ferromagnetic material consisting essentially of crystals of a composition having the formula:



in which

$\text{M}^{\text{II}}$  is at least one divalent metal selected from the group consisting of Mn, Fe, Co, Ni, Cu, Zn, and Mg, and

$a$  has a value less than 0.5

$(b+c)$  has a value less than 0.25

$(e+f)$  has a value less than 0.6

70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 682

ing of a highly-coherent mass of crystals of a composition having the formula:



in which

$\text{M}^{\text{II}}$  is at least one divalent metal selected from the group consisting of Mn, Fe, Co, Ni, Cu, Zn, and Mg, and

$a$  has a value less than 0.5

$(b+c)$  has a value less than 0.25

$(e+f)$  has a value less than 0.6

said crystals having a rhombohedral structure, of which the unit cell in the hexagonal crystal can be described with a  $c$ -axis of about 43.5 Å. and an  $a$ -axis of about 5.9 Å.

3. A permanent magnet comprising a magnetized highly-coherent body consisting essentially of crystals of a composition having the formula:



in which

$\text{M}^{\text{II}}$  is at least one divalent metal selected from the group consisting of Mn, Fe, Co, Ni, Cu, Zn, and Mg, and

$a$  has a value less than 0.5

$(b+c)$  has a value less than 0.25

$(e+f)$  has a value less than 0.6

said crystals having a rhombohedral structure of which the unit cell in the hexagonal crystal system can be described with a  $c$ -axis of about 43.5 Å. and an  $a$ -axis of about 5.9 Å.

4. A method of producing a ferromagnetic material which comprises the steps, forming a finely-divided mixture of oxides in proportions forming upon heating crystals of a composition having the formula:



in which

$\text{M}^{\text{II}}$  is a divalent metal selected from the group consisting of Mn, Fe, Co, Ni, Cu, Zn, and Mg, and

$a$  has a value less than 0.5

$(b+c)$  has a value less than 0.25

$(e+f)$  has a value less than 0.25,

said crystals having a rhombohedral structure, of which the unit cell in the hexagonal system can be described with a  $c$ -axis of about 43.5 Å. and an  $a$ -axis of about 5.9 Å.; and heating said mixture in an atmosphere containing at least as much oxygen as air at a temperature of about 1000° to 1300° C. for a time sufficient to form said crystals.

5. A method of producing a ferromagnetic material comprising the steps, forming a finely-divided mixture of divalent metal oxides and ferric oxide in proportions yielding upon heating crystals having a structure corresponding to that of the mineral magnetoplumbite; heating said mixture at a temperature below 1100° C. and sufficiently high to form said crystals; mixing said crystals with additional oxides of divalent metals in amounts sufficient to form upon heating crystals of a composition having the formula:



in which

$\text{M}^{\text{II}}$  is a divalent metal selected from the group consisting of Mn, Fe, Co, Ni, Cu, Zn, and Mg, and

$a$  has a value less than 0.5

$(b+c)$  has a value less than 0.25

$(e+f)$  has a value less than 0.6,

said latter crystals having a rhombohedral structure, of which the unit cell in the hexagonal system can be described with a  $c$ -axis of about 43.5 Å. and an  $a$ -axis of about 5.9 Å.; and heating the latter mixture in an atmosphere containing at least as much oxygen as air to a tem-

perature of about 1000° to 1300° C. for a time sufficient to form said latter crystals.

6. A method of producing a ferromagnetic material comprising the steps, forming a finely-divided mixture of divalent metal oxides in proportions forming upon subsequent heating crystals of a composition having the formula:



10 in which

$\text{M}^{\text{II}}$  is a divalent metal selected from the group consisting of Mn, Fe, Co, Ni, Cu, Zn, and Mg, and

$a$  has a value less than 0.5

$(b+c)$  has a value less than 0.25

$(e+f)$  has a value less than 0.6,

said crystals having a rhombohedral structure, of which the unit cell can be described with a  $c$ -axis of about 43.5 Å. and an  $a$ -axis of about 5.9 Å.; heating said mixture to a temperature between about 900° to 1200° C. to react the same; finely-dividing the reaction product; and heating the finely-divided reacted product in an atmosphere containing at least as much oxygen as air to a temperature of about 1000° to 1300° C. for a time sufficient to form said crystals.

7. A method of producing a ferromagnetic body which comprises the steps forming a finely-divided mixture of oxides in proportions forming upon heating crystals of a composition having the formula:



in which

$\text{M}^{\text{II}}$  is a divalent metal selected from the group consisting of Mn, Fe, Co, Ni, Cu, Zn, and Mg, and

$a$  has a value less than 0.5

$(b+c)$  has a value less than 0.25

$(e+f)$  has a value less than 0.25,

said crystals having a rhombohedral structure, of which the unit cell in the hexagonal system can be described with a  $c$ -axis of about 43.5 Å. and an  $a$ -axis of about 5.9 Å.; compacting said mixture into a body of desired shape and dimensions; and heating said compacted body in an atmosphere containing at least as much oxygen as air at a temperature of about 1000° to 1300° C. for a time sufficient to form said crystals.

8. A method of producing a permanent magnet body which comprises the steps forming a finely-divided mixture of oxides in proportions forming upon heating crystals of a composition having the formula:



in which

$\text{M}^{\text{II}}$  is a divalent metal selected from the group consisting of Mn, Fe, Co, Ni, Cu, Zn, and Mg, and

$a$  has a value less than 0.5

$(b+c)$  has a value less than 0.25

$(e+f)$  has a value less than 0.25,

said crystals having a rhombohedral structure, of which the unit cell in the hexagonal system can be described with a  $c$ -axis of about 43.5 Å. and an  $a$ -axis of about 5.9 Å.; compacting said mixture into a body of desired shapes and dimensions; heating said compacted body in an atmosphere containing at least as much oxygen as air at a temperature of about 1000° to 1300° C. for a time sufficient to form said crystals; and magnetizing said body in a strong magnetic field.

70 References Cited in the file of this patent

UNITED STATES PATENTS

2,659,698 Berge Nov. 17, 1953

(Other references on following page)

## UNITED STATES PATENTS

2,723,239 Harvey Nov. 8, 1955  
 2,736,708 Crowley Feb. 28, 1956  
 2,762,777 Went Sept. 11, 1956  
 2,762,778 Gorter et al. Sept. 11, 1956  
 2,778,803 Crowley Jan. 22, 1957  
 2,828,264 Medvedieff Mar. 25, 1958

## FOREIGN PATENTS

1,100,865 France Apr. 13, 1955

927,259 Germany May 2, 1955  
 165,447 Australia Oct. 4, 1955

## OTHER REFERENCES

Erchak et al.: J. Amer. Chem. Soc., October 1946,  
 pp. 2085-2093.

Harvey et al.: RCA Review, September 1950, p. 346.  
 "Phillips Technical Review," vol. 13, No. 7, pp.  
 194-208.

"Phillips Technical Review," vol. 18, No. 6, pp.  
 145-154.

UNITED STATES PATENT OFFICE  
CERTIFICATE OF CORRECTION

Patent No. 2,946,753

July 26, 1960

Gerard Heinrich Jonker et al.

It is hereby certified that error appears in the printed specification of the above numbered patent requiring correction and that the said Letters Patent should read as corrected below.

Column 2, line 13, for "coaxis" read -- c-axis --; line 14, for "an axis" read -- an a-axis --; line 57, for "pentonite" read -- bentonite --; column 7, line 16, and column 8, line 47, for "permanent magnet", each occurrence, read -- ferromagnetic body --.

Signed and sealed this 10th day of January 1961.

(SEAL)

Attest:

KARL H. AXLINE

Attesting Officer

ROBERT C. WATSON  
Commissioner of Patents